

## UNITED STATES PATENT OFFICE

1,944,529

## FLOTATION PROCESS

Wilhelm Schäfer and Willy Mertens, Bochum, Germany, assignors to Erz- und Kohle-Flotation Gesellschaft mit beschränkter Haftung, Bochum, Germany

No Drawing. Application January 11, 1933, Serial No. 631,228, and in Germany September 26, 1931

16 Claims. (Cl. 209—166)

This invention relates to froth-flotation of coal, for the purpose to separate the fusain from the other structural constituents of coal namely vitrain, clarain and durain.

According to the United States Patent No. 1,499,872, it is known to render the fusain, which is present in nearly all coals and has an adverse influence on coking, wettable and nonfloatable by the addition of protective colloids such as starch, tannin, albumen or glue, to the coal slurry in the preparation of the coal by the flotation process, whereby it is necessary to regulate the amount of said protective colloids so that the other structural constituents of the coal retain their floatable capacity and can be floated out as a product low in fusain. These processes have the drawback of being extremely delicate, in consequence of which the separation of the fusain from the other structural constituents of the coal is usually incomplete. If, for example, the requisite concentration of the protective colloids be slightly exceeded, the depressing action of the protective colloids extends, to a certain extent, to the vitrain and durain which then partly pass away together with the fusain. If the concentration of the protective colloids be too low, a portion of the fusain will be left in the vitrain and the desired degree of separation will not be attained.

The object of the present invention is to provide a flotation process enabling the separation of the fusain from the other structural constituents to be effected in a less delicate and more complete manner.

According to this invention fusain is separated from the other constituents of coal in a froth-flotation process by adding to the pulp in presence of a froth producing reagent a protective colloid which depresses the durain, vitrain and clarain without affecting the floatability of fusain. The protective colloids which can be used in carrying out this invention may be polyhexoses  $[(\text{CeH}_{10}\text{O}_5)_x]$  such as starches or dextrins] which have been pre-treated with hydrogen-chloride. The most effective result can be obtained in treating starches or dextrins with hydrogen-chloride in nascent state by adding agents which split off hydrogen-chloride when treated with water. These agents may be organic acid chlorides (such as acetylchloride and benzoylchloride) or some suitable inorganic chlorides (such as  $\text{AlCl}_3$  and  $\text{ZnCl}_3$ ).

It has been ascertained that starches or dextrins, pre-treated in the described manner, form suitable additions which do not affect the float-

ability of the fusain, but on the other hand, exert a powerful depressing action on the vitrain and durain constituents. The advantage of the new process resides both in the less delicate adjustment of the quantities of the added agents, and in the attainment of a substantial improvement in the degree of separation. Inasmuch as the fusain retains its floatability even when the amounts of pre-treated dextrins and starches exceed those required to effect the depression of the vitrain and durain constituents, it can be extensively floated off after adding a frothing agent, whilst the other structural constituents of the coal remain unfloatable. The froth producing agents which can be used for the separation of the fusain may preferably be wood-tar oils of low boiling point (105-160° Cels.) whilst wood-tar oils of higher boiling point would partly neutralize the depressing action of the protective colloids.

After separating the froth containing the fusain, the remaining pulp after the addition of a slightly dissociated alkali and one or more suitable frothing agents is subjected to a second froth-flotation operation adapted to separate the durain, vitrain and clarain from the waste. The addition of a slightly dissociated alkali to the pulp after the removal of the fusain has the effect of again rendering the other structural constituents floatable. These constituents can then be floated off as a product that is low in ash and practically free from fusain with the result that the recovery can be raised to a maximum because there is no longer any need to take into consideration the chance of fusain being floated off with the said constituents.

In carrying out the process, the coal slurry to be subjected to flotation is treated, prior to the addition of the flotation oil, with the aqueous solution of 100-300 grams, according to the kind of coal, of dextrins or starches that have been pre-treated with hydrogen-chloride, inorganic chlorides or organic acid chlorides, whereupon the added agent having been intimately mixed with the coal slurry, a wood-tar oil of low boiling point is added. The slurry is then agitated by pneumatic or mechanical means in known manner and the resulting froth containing the fusain in a concentrated condition is removed while the other structural constituents of the coal remain in the pulp. After the fusain has been removed, the slurry is treated with slightly dissociated alkalies, such as sodium carbonate or waterglass, until dye reaction is neutral or slightly alkaline. Finally, the other structural constituents are

floated off by the addition of the known oils suitable for coal flotation.

The manner in which the polyhexose pre-treated with hydrogen-chloride, act in the separation of the fusain from the other structural constituents of the coal, by the flotation process, will be evident from the following examples:—

*Example 1.*—1000 grams of coal slurry from a Ruhr colliery and with a solid:liquid ratio of 1:4, were treated with 0.2 grams of dextrin (pre-treated with hydrogen-chloride) and, after stirring for several minutes, floated with addition of 3 drops of hard-wood tar oil boiling at 120/160° Cels. After removing the fusain product, the residual slurry was treated with 0.2 grams of sodium carbonate and floated, with an addition of creosote as a vitrain and durain product. The recovered products are set out in the following table:

| Product             | Weight (%) | Ash (%) | Ash (kgs.) |
|---------------------|------------|---------|------------|
| Fusain product..... | 6.1        | 15.8    | 0.96       |
| Coal.....           | 37.5       | 8.8     | 3.30       |
| Middlings.....      | 14.1       | 35.2    | 4.97       |
| Waste.....          | 42.3       | 59.8    | 25.34      |
| Raw coal.....       | 100.0      | 34.2    | 34.57      |

The fusain product has no caking capacity and cannot be coked. On the other hand, the coal product exhibits excellent caking capacity and furnishes a firm microporous coke.

*Example 2.*—1000 grams of dust coal from an English coal deposit were stirred for several minutes with about 3 parts of water and the addition of 0.15 grams of starch (pre-treated with acetyl chloride), and then floated with the addition of 4 drops acetone-light oil (boiling point 105°-140° Cels.). After the removal of a fusain product, as the first batch of foam, the vitrain and fusain were floated off with addition of 0.3 grams of waterglass and 4 drops of cresol. The following products were separated from 100 parts of the dust coal.

| Products            | Weight (%) | Ash(%) | Ash (kgs.) |
|---------------------|------------|--------|------------|
| Fusain product..... | 18.8       | 7.8    | 1.47       |
| Coal.....           | 57.6       | 5.5    | 3.17       |
| Middlings.....      | 9.8        | 13.4   | 1.31       |
| Waste.....          | 13.8       | 59.1   | 8.15       |
| Raw coal.....       | 100.0      | 14.1   | 14.10      |

The fusain product exhibited poor caking capacity whilst on the other hand, that of the coal product was very good.

*Example 3.*—In the flotation of a slurry of Silesian coal the fusain product was first floated off, with addition of 0.2 grms. of dextrin (pre-treated with zinc-chloride), the flotation of the vitrain and fusain constituents being then effected after addition of 0.4 grms of waterglass and 5 drops of coaltar oil. The results are given in the following table:—

| Product             | Weight (%) | Ash (%) | Ash.(kgs.) |
|---------------------|------------|---------|------------|
| Fusain product..... | 13.5       | 10.5    | 1.42       |
| Coal.....           | 51.5       | 6.8     | 3.51       |
| Middlings.....      | 21.8       | 19.2    | 4.18       |
| Waste.....          | 13.2       | 69.1    | 9.12       |
| Raw coal.....       | 100.0      | 18.1    | 18.23      |

The recovered fusain product cannot be coked, whereas the coal product furnishes excellent coke. It is evident from the above example that the

new flotation process is generally applicable to the separation of the fusain from the other structural constituents of coal. In addition to the examples given, in which coals from the Ruhr, Silesian and English coal districts were treated, experiments were also conducted with coal from Saxony, the Sarre district and Czechoslovakia, and furnished similar good results in respect of separation.

The quantity of pre-treated dextrans and starches required for carrying out the process ranges in general, between 100 and 300 grams per ton of raw coal, though, if necessary, it may be increased up to 500 grams per ton of raw coal.

Having now particularly described certain embodiments of our invention,

We claim:

1. A flotation process for separating fusain from the other structural constituents of coal, wherein heterogeneous coal is made into a pulp with water and subjected to froth-flotation separation in the presence of a froth producing reagent and of a polyhexose which has been pre-treated with hydrogen-chloride. 95

2. A flotation process for separating fusain from the other structural constituents of coal, wherein heterogeneous coal is made into a pulp with water and subjected to froth-flotation separation in the presence of a froth producing reagent and of a polyhexose which has been pre-treated with hydrogen-chloride in nascent state 105 by adding agents which split off hydrogen-chloride when treated with water.

3. A flotation process for separating fusain from the other structural constituents of coal, wherein heterogeneous coal is made into a pulp with water and subjected to froth-flotation separation in the presence of a froth producing reagent and of a polyhexose which has been pre-treated with inorganic chlorides which split off 115 hydrogen-chloride when treated with water.

4. A flotation process for separating fusain from the other structural constituents of coal, wherein heterogeneous coal is made into a pulp with water and subjected to froth-flotation separation in the presence of a froth producing reagent and of a polyhexose which has been pre-treated with organic acid chlorides. 120

5. A flotation process for separating fusain from the other structural constituents of coal, wherein coal is made into a pulp with water and subjected to a froth-flotation separation in the presence of a froth producing reagent and of starch which has been pre-treated with 125 hydrogen-chloride.

6. A flotation process for separating fusain from the other structural constituents of coal, wherein coal is made into a pulp with water and subjected to a froth-flotation separation in the presence of a froth producing reagent and of starch which has been pre-treated with 135 hydrogen-chloride in nascent state by adding agents which split off hydrogen-chloride when treated with water.

7. A flotation process for separating fusain from the other structural constituents of coal, wherein coal is made into a pulp with water and subjected to a froth-flotation separation in the presence of a froth producing reagent and of starch which has been pre-treated with 145 inorganic chloride which split off hydrogen-chloride when treated with water.

8. A flotation process for separating fusain from the other structural constituents of coal, 150

- wherein coal is made into a pulp with water and subjected to a froth-flotation separation in the presence of a froth producing reagent and of starch which has been pre-treated with organic acid chlorides. 5
9. A flotation process for separating fusain from the other structural constituents of coal, wherein heterogeneous coal is made into a pulp with water and subjected to a froth-flotation operation in the presence of a froth producing reagent and of dextrins which has been pre-treated with hydrogen-chloride. 10
10. A flotation process for separating fusain from the other structural constituents of coal, wherein heterogeneous coal is made into a pulp with water and subjected to a froth-flotation operation in the presence of a froth producing reagent and of dextrins which has been pre-treated with hydrogen-chloride in nascent state 15 by adding means which split off hydrogen-chloride when treated with water. 20
11. A flotation process for separating fusain from the other structural constituents of coal, wherein heterogeneous coal is made into a pulp with water and subjected to a froth-flotation operation in the presence of a froth producing reagent and of dextrins which has been pre-treated with inorganic chlorides which split off hydrogen-chloride when treated with water. 25
12. A flotation process for separating fusain from the other structural constituents of coal, wherein heterogeneous coal is made into a pulp with water and subjected to a froth-flotation operation in the presence of a froth producing reagent and of dextrins which has been pre-treated with organic acid chlorides. 30
13. A flotation process for separating fusain from the other structural constituents of coal, wherein heterogeneous coal is made into a pulp with water and subjected to a froth-flotation operation in the presence of a small quantity 40
- of wood-tar oil of low boiling point and of a polyhexose which has been pre-treated with hydrogen-chloride. 5
14. A flotation process for separating fusain from the other structural constituents of coal, wherein heterogeneous coal is made into a pulp with water and subjected to a froth-flotation operation in the presence of a froth producing reagent and of a polyhexose which has been pre-treated with hydrogen-chloride; separating the froth containing the fusain and adding to the remaining pulp slightly dissociated alkalis for the purpose of again rendering the other structural constituents floatable. 80
15. A flotation process for separating fusain from the other structural constituents of coal, wherein heterogeneous coal is made into a pulp with water and subjected to a froth-flotation operation in the presence of a small quantity of wood-tar oil of low boiling point and of a polyhexose which has been pre-treated with hydrogen-chloride; separating the froth containing the fusain and adding to the remaining pulp slightly dissociated alkalis for the purpose of again rendering the other structural constituents floatable. 85
16. A flotation process for separating fusain from the other structural constituents of coal, wherein heterogeneous coal is made into a pulp with water and subjected to a froth-flotation operation in the presence of a froth producing reagent and of a polyhexose which has been pre-treated with hydrogen-chloride; separating the froth containing the fusain and again subjecting the remaining pulp after the addition of a slightly dissociated alkali and a frothing agent to a flotation operation to separate the durain, clarain and vitrain from the waste. 95
- 120
- WILHELM SCHÄFER. 115  
WILLY MERTENS.
- 45
- 50
- 55
- 60
- 65
- 70
- 75
- 125
- 130
- 135
- 140
- 145
- 150